

1

2,984,587

## TEXTILE SOFTENING AGENTS AND METHOD OF APPLYING THEM

Erich Matter, Riehen, Otto Albrecht, Neue-Welt, and Armin Hiestand, Binningen, Switzerland, assignors to Ciba Limited, Basel, Switzerland

No Drawing. Filed Jan. 20, 1959, Ser. No. 787,832

Claims priority, application Switzerland Jan. 14, 1957

10 Claims. (Cl. 117—139.5)

The present invention is a continuation-in-part of our application Serial No. 706,281, filed December 31, 1957 (abandoned since the filing of the present application), and relates to new textile softening agents and a method of applying them.

According to the present invention a soft handle and feel can be imparted to textile material by contacting the material with an aqueous bath containing a di-quaternary ammonium compound of the general formula



in which R<sub>1</sub> and R<sub>1'</sub> each represents high molecular aliphatic hydrocarbon radicals, especially an alkyl radical having from 10 to 18 carbon atoms, R<sub>2</sub>, R<sub>2'</sub>, R<sub>3</sub> and R<sub>3'</sub> represent the same or different aliphatic, cycloaliphatic, araliphatic or aromatic radicals, in which R<sub>2</sub> and R<sub>3</sub>, and/or R<sub>2'</sub> and R<sub>3'</sub> may together constitute a divalent aliphatic radical, R<sub>4</sub> and R<sub>4'</sub> represent alkylene radicals, R<sub>5</sub> represents a divalent aliphatic or aromatic radical, R<sub>6</sub> and R<sub>6'</sub> represent a hydrogen atom or a low molecular aliphatic radical, and X represents an anion.

As the radicals R<sub>2</sub>, R<sub>2'</sub>, R<sub>3</sub> and R<sub>3'</sub> there come into consideration, more especially, low molecular alkyl- and hydroxylalkyl groups, also high molecular aliphatic hydrocarbon radicals, as, for example, alkyl radicals having from 10 to 18 carbon atoms.

The invention is concerned, more especially, with compounds of the general symmetrical formula



in which R<sub>1</sub>, R<sub>2</sub>, R<sub>3</sub>, R<sub>4</sub> and R<sub>5</sub> and X have the meanings given above.

The compounds of the above mentioned Formulas I and II in which R<sub>2</sub> and R<sub>2'</sub> and, if desired, R<sub>3</sub> and R<sub>3'</sub>, have the same meaning as R<sub>1</sub> and R<sub>1'</sub>, that is, they represent a high molecular aliphatic hydrocarbon radical, are especially valuable softening agents for cellulose-containing or synthetic textile fibrous materials as, for example, cotton, regenerated cellulose acetate silk, nylon, polyethylene terephthalate and especially polyacrylonitrile.

Especially advantageous as softening agents are the compounds of the formula

2



in which R<sub>1</sub> and R<sub>2</sub> represent straight-chain alkyl group containing 10 to 18 carbon atoms, R<sub>3</sub> each represents an aliphatic radical containing 1 to 4 carbon atoms, and m and n represent small whole numbers.

Among these compounds there are preferred those in which m in the above formula is 1, 2 or 3, especially 1, and n is 1.

The compounds can be obtained by known methods. For instance 2 mols of a compound of the formula



may be quaternised with 1 mol of a compound of the formula



in which X represents a substituent capable of forming an anion, especially a halogen atom.

As tertiary amines of the Formula 1 there may be mentioned, for example, dimethyl-dodecyl amine, dimethyl-cetylamine, dimethyl-octadecyl amine, diethyl-dodecyl amine, dipropyl-dodecyl amine, dibutyl-dodecyl amine, di-hydroxyethyl dodecyl amine, N:N-dimethyl-para-dodecyl aniline, didodecyl-methyl amine, dicetyl-methyl amine and dioctadecyl-methyl amine.

The diamides of the Formula 2 may themselves be prepared by the condensation of 1 mol of a diprimary di- or poly-amine of the formula



with 2 mols of a halogeno-fatty acid, or a functional derivative thereof, for example, chloracetic acid or chloroacetic acid methyl ester.

The diamides of the Formula 2 in which R<sub>5</sub> represents a radical



in which R<sub>7</sub> represents H, —CH<sub>3</sub> or —C<sub>6</sub>H<sub>5</sub>) are obtained by the condensation of 2 mols of an N-methylolamide of the formula



or by means of a catalytic reaction of an aldehyde such as formaldehyde, acetaldehyde or benzaldehyde with acrylonitrile (or its homologues), hydrochloric acid and steam in the gaseous phase.

According to a further process 2 mols of a compound of the formula



may be condensed with a compound of the formula



with splitting off of hydrogen halide and the condensation product so obtained is then treated with a quaternating agent of the formula R<sub>3</sub>—X. As such quaternating

agents there may be mentioned, for example, dimethylsulfate and methyl iodide.

In a yet further process 2 mols of a compound of the formula



or a functional derivative thereof, such as acid anhydride, 10 acid ester or acid halide, may be condensed with 1 mol of a dipimary di- or poly-amine of the formula



The monoquaternary ammonium compounds of the 15 Formula 4 can themselves be obtained by quaternating a tertiary amine of the formula



with a halogeno-fatty acid or functional derivative thereof, as, for example, chloracetic acid or chloracetic acid methyl ester.

As dipimary di- or poly-amines there come into consideration, for example, propylene-diamine, hexamethylene diamine, diethylene-triamine, N-di(2-aminoethyl)-N-methyl-amine, 1:4-phenylene diamine and especially ethylene diamine.

Furthermore, it is also possible to condense 2 mols of 30 a tertiary amine of the formula



or a functional derivative of such a carboxylic acid, with a dipimary di- or poly-amine, and then treat the di-tertiary amine so obtained with 2 mols of a quaternating agent of the formula  $\text{R}_3\text{X}$ . As such quaternating agents there may be mentioned, for example, dodecyl bromide and octadecyl bromide.

Instead of the amines of Formula 5 there may be used those of the formula



or a functional derivative thereof, and with the use of a 50 quaternating agent of the formula  $\text{R}_3\text{X}$ .

As such quaternating agents there may be mentioned, for example, dimethyl sulfate, ethyl bromide, ethyl iodide and benzyl chloride.

According to a further method 2 mols of a diamine of the formula



may be condensed with 1 mol of a dicarboxylic acid of the formula



or a functional derivative thereof, such as acid anhydride, 65 ester or acid halide, and the di-tertiary amine so obtained is treated with 2 mols of a quaternating agent of the formula  $\text{R}_1\text{X}$ .

As diamines of the Formula 7 there may be mentioned, for example, N:N-dimethyl ethylene diamine, N:N-di-methyl propylene diamine and N:N-diethyl ethylene diamine.

As dicarboxylic acids there come into consideration malonic acid, glutaric acid, adipic acid, maleic acid, fumaric acid, butadiene-1:4-dicarboxylic acid, tereph-

thalic acid, 1:4-naphthalene dicarboxylic acid and especially succinic acid, or their esters or acid halides.

Instead of diamine of the Formula 7 there may be used one of the formula



and as quaternating agent one of the formula  $\text{R}_3\text{X}$ .

The following examples illustrate the invention, the parts being by weight:

#### Example 1

Polyacrylonitrile yarn ("Orlon" yarn type 42) was treated at 30° C. for half an hour and at a goods-to-liquor ratio of 1:30, with a solution which contained 0.08% of the product described below calculated on the weight of the fibrous material. The yarn so treated possessed a very soft handle, which even after washing with a synthetic washing agent at 40° C. was only slightly impaired.

The product used in this example may be prepared as follows:

43 grams of dimethyl-dodecyl amine and 21.2 grams of a compound which had been obtained by condensation in the molecular ratio of 2:1 of chloracetic acid methyl ester with ethylene-diamine, were stirred for 5 hours at 100° C.

There was obtained a light paste which was stirred with 400 ccs. of water-free ether. After suction-filtering in the cold there was obtained a colorless, wax-like mass. This product, which corresponds to the formula



was a clear, water-soluble compound which was stable to sodium carbonate.

The quaternating reaction may also be carried out in aqueous solution. In this case the mixture was more easily stirrable.

#### Example 2

The process described in Example 1 was carried out 45 but with the use of a polyamide fiber, for example, nylon yarn. The textile material so treated possessed a very soft handle.

In a similar manner cotton yarn may also be treated.

#### Example 3

A polyester yarn (from terephthalic acid and glycol) was treated at 30° C. for half an hour, and at a goods-to-liquor ratio of 1:30, with a solution which contained 0.4% of the quaternary salt described below, calculated on the weight of the yarn. The fibrous material so treated was substantially softer to the touch than the untreated material.

The product used in this example may be prepared as follows:

60 A mixture of 30 grams of the commercially known tertiary amine of the formula



in which R represents the alkyl radical derived from hydrogenated tall oil fatty acid, and 5.3 grams of N:N'-methylene-bis-(chloracetamide) of the formula



was stirred for 6 hours on a boiling water bath while 75 passing nitrogen through the apparatus. The di-quater-

inary ammonium salt so obtained, which corresponded to the formula



was a wax-like mass which with hot water yielded an opalescent solution.

*Example 4*

Viscous yarn was treated at 30° C. for half an hour at a goods-to-liquor ratio of 1:30 with a solution containing 0.3% (based on the weight of the yarn) of the product described below. The yarn so treated possessed a very fine soft handle.

The product used in this example may be prepared as follows:

88 grams (0.2 mol) of a dialkylamine of the formula



5

2. The di-quaternary ammonium compound which corresponds to the formula



10

in which  $\text{R}_1$  and  $\text{R}_2$  each represents a straight-chain alkyl radical containing from 10 to 18 carbon atoms,  $\text{R}_3$  represents an alkyl radical containing from 1 to 4 carbon atoms,  $m$  and  $n$  are small whole numbers and  $\text{X}$  represents the anion of a water-soluble inorganic acid.

3. The di-quaternary ammonium compound which corresponds to the formula



20

in which  $\text{R}_1$  and  $\text{R}_2$  each represents a straight-chain alkyl radical containing from 10 to 18 carbon atoms,  $\text{R}_3$  represents an alkyl radical containing from 1 to 4 carbon atoms,  $m$  and  $n$  are small whole numbers and  $\text{X}$  represents the anion of a water-soluble inorganic acid.

4. The compound of the formula



wherein  $\text{R}$  represents the alkyl radical derived from hydrogenated tall oil fatty acid.

5. The compound of the formula



wherein  $\text{R}$  represents the alkyl radical derived from coconut oil fatty acid.

6. A process for imparting a soft handle and feeling to textile material which comprises impregnating the material in an aqueous bath containing the di-quaternary ammonium compound which corresponds to the general symmetrical formula



55 in which  $\text{R}_1$  represents an aliphatic hydrocarbon radical containing from 10 to 18 carbon atoms,  $\text{R}_2$  and  $\text{R}_3$  each represents an aliphatic hydrocarbon radical containing from 1 to 4 carbon atoms,  $\text{R}_4$  and  $\text{R}_5$  each represents an alkylene radical, and  $\text{X}$  represents the anion of a water-soluble inorganic acid.

60 7. A process for imparting a soft handle and feeling to textile material which comprises impregnating the material in an aqueous bath containing the di-quaternary ammonium compound which corresponds to the formula



65 in which  $\text{R}_1$  and  $\text{R}_2$  each represents a straight-chain alkyl radical containing from 10 to 18 carbon atoms,  $\text{R}_3$  represents an alkyl radical containing from 1 to 4 carbon atoms,  $m$  and  $n$  are small whole numbers and  $\text{X}$  represents the anion of a water-soluble inorganic acid.

70 75

atoms,  $m$  and  $n$  are small whole numbers and  $X$  represents the anion of a water-soluble inorganic acid.

8. A process for imparting a soft handle and feeling to textile material which comprises impregnating the material in an aqueous bath containing the compound of the formula 5



10

wherein  $R$  represents the alkyl radical derived from hydrogenated tall oil fatty acid.

9. A process for imparting a soft handle and feeling to textile material which comprises impregnating the material in an aqueous bath containing the compound of the formula 15



20

wherein  $R$  represents the alkyl radical derived from coconut oil fatty acid.

10. A process for imparting a soft handle and feeling to textile material which comprises impregnating the material in an aqueous bath containing the compound of the formula 25



References Cited in the file of this patent

UNITED STATES PATENTS

|           |                      |                |
|-----------|----------------------|----------------|
| 2,176,896 | Epstein et al.       | Oct. 24, 1939  |
| 2,216,406 | Austin               | Oct. 1, 1940   |
| 2,310,873 | Sauer                | Feb. 9, 1943   |
| 2,334,709 | Katzman et al.       | Nov. 23, 1943  |
| 2,371,104 | Kienle et al.        | Mar. 6, 1945   |
| 2,569,409 | De Benneville et al. | Sept. 25, 1951 |
| 2,653,898 | Castillo et al.      | Sept. 29, 1953 |
| 2,669,582 | Cusic                | Feb. 16, 1954  |
| 2,765,337 | De Benneville et al. | Oct. 2, 1956   |
| 2,832,799 | Payne et al.         | Apr. 29, 1958  |

FOREIGN PATENTS

|           |             |               |
|-----------|-------------|---------------|
| 210,482   | Switzerland | July 15, 1940 |
| 748,543   | Germany     | Nov. 17, 1944 |
| 1,110,724 | France      | Oct. 19, 1955 |
| 936,395   | Germany     | Dec. 15, 1955 |

OTHER REFERENCES

Phillips: Jour. Am. Chem. Soc., vol. 73, pages 5822-5824.

UNITED STATES PATENT OFFICE  
CERTIFICATION OF CORRECTION

Patent No. 2,984,587

May 16, 1961

Erich Matter et al.

It is hereby certified that error appears in the above numbered patent requiring correction and that the said Letters Patent should read as corrected below.

Column 5, lines 65 and 66, the lower left-hand portion of the formula should appear as shown below instead of as in the patent:



column 6, lines 18 to 25 and lines 65 to 72, the closing bracket, each occurrence, should appear as shown below instead of as in the patent:



column 7, lines 8 and 28, after the closing bracket, for "C<sub>12</sub><sup>⊖</sup>", each occurrence, read -- 2C<sub>1</sub><sup>⊖</sup> --.

Signed and sealed this 31st day of October 1961.

(SEAL)

Attest:

ERNEST W. SWIDER  
Attesting Officer

DAVID L. LADD  
Commissioner of Patents